

Patented Jan. 22, 1929.

1,699,683

# UNITED STATES PATENT OFFICE.

HERMAN J. BIEFANG, OF CINCINNATI, OHIO.

## PROCESS FOR TREATING STEEL.

No Drawing.

Application filed May 7, 1923. Serial No. 637,353.

My invention relates to processes of treating metals adapted for use as high speed cutting tools, and has to do more particularly with such a process adapted for treating so-called high speed steels, an object being to improve the steel to make it susceptible to better hardening.

Another object of my invention is to so treat the steel that when used for tools, such as machine cutting tools, they have greater wearing qualities, and many other advantages hereinafter more particularly pointed out.

Generally speaking, my improved process consists of heat treating, high speed steel or metal, or metal used for high speed cutting tools so as to improve it in various ways and make it more susceptible to better hardening. To this end, the steel is immersed in a bath of molten metal of such character and temperature, that it acts upon the steel as to improve its qualities as stated above, and so far as I am able to observe forms an incrustation on the metal which appears when it is withdrawn from the bath.

I have found that high speed steel treated according to my process, produces astonishing results in that there is less brittleness of the cutting edges of the tool, greater resistance to wear, and extension of the life of the tool, in that less grinding is necessary.

More particularly in employing my process in its preferred form, I provide a bath for the tool in the form of molten lead and preferably add a small portion of copper to prevent burning of the lead by reason of the high temperature of the bath.

I find that seven parts of lead to one part of copper, serves the purpose very well, heating them sufficiently to form an alloy. This mixture used as a bath is heated from a melting or fusing temperature of the composition to 1800 degrees Fahrenheit for treating the steel. While heating the metal, I preferably place a layer of crushed charcoal over the top, and this must be refreshed or it becomes foul, apparently with the sulphur extracted from the steel being treated. A slight addition of such alloy and charcoal every time the bath is used, will overcome this fouling difficulty.

I now place the tool of high speed steel, or the piece to be treated, in the bath so that it is below the surface, avoiding contact of the cutting edges of the tool with the crucible, so that the fluid of the bath uniformly covers the steel.

I find that the higher temperature produces a quicker operation in that the bubbling and incrustation upon the steel is produced in a shorter period of time, but there is always the danger of the high temperature in that it may possibly absorb some of the metals comprising the various constituents of high speed steel. For this reason a lower temperature is more desirable, and I find that a temperature just above the melting point of the composition works very well.

At the high heat treatment, that is closer to 1800 degrees, I find that after the steel is heated five minutes or so, what apparently is a sulphurous smoke, rises from the steel and accumulates as an incrustation on the outside of the steel. At the lower heat treatment, with a tool made up of bar steel one inch by one-half inch, smoke will issue in about ten minutes and the treatment evidently is well completed in about twenty minutes.

I find that it is desirable to drop the temperature of the bath to closely above the fusing point while treating the steel and before it is removed from the bath. The steel after being removed from the bath and cooled should be cleaned by removing the incrustation on the surface, preferably by using an ordinary scraper or a wire brush. It is then ready to be hardened if required in any of the well known ways.

I find that when immersing the metal which is to be treated in the heat bath, the bath will bubble like boiling water, the bubbling varying with different pieces being immersed. This difference in the boiling apparently arises from differences in the amount of undesirable or foreign substances in the metal which is being treated.

Tools when forged and still hot may be placed in the bath, but under such conditions it is desirable that they be below the temperature of the bath so as to avoid placing a contractual strain on the tool, due to the bath acting as a cooling agent. The tools may, however, be placed in the bath when cold and left in long enough to complete the treatment by becoming heated through and then "soaking" for ten minutes or more depending upon the size of the piece being treated, until a smoke arises from the tool and an incrustation forms on the surface, when it is removed from the bath and exposed to the air.

What I claim as new and desire to secure by United States Letters Patent is:

1. The process of treating cutting tool metal to make it susceptible to better hardening consisting of immersing a piece of high speed steel or other cutting metal in a molten metal bath of substantially seven parts lead and one part copper at a temperature above fusing of the bath, leaving the steel in the bath long enough to have the surface of the piece covered with a sediment formed in the bath, and then gradually cooling the steel after withdrawing it from the bath. 5
2. The process of treating metal to make it susceptible to better hardening consisting of immersing a piece of high speed cutting tool metal in a molten metal bath of lead and copper at a temperature of approximately 1800 degrees Fahrenheit, and leaving the piece in the bath sufficiently long enough to assume the temperature of the bath and also 10 have the surface of the piece incrusted with a sediment formed thereby. 15
3. The process of treating metal consisting of immersing the metal in a molten metal bath comprising lead and a sufficient quantity of copper to prevent burning of the lead while at a temperature sufficient to treat the metal, the temperature of the bath being preferably sufficient to form an incrustation on 20 the treated metal, leaving the metal in the bath long enough to have the surface of the piece 25 incrusted with a sediment formed in the bath, then cooling the metal and cleaning its surface for further desired treatment. 30
4. The process of treating metal or cutting metals consisting of immersing a piece of high speed cutting tool metal to be formed as a tool in a molten metal bath comprising approximately seven parts lead and one part copper at a temperature above the fusing temperature of the bath but low enough to prevent absorbing any of the metal constituents of the treated metal, leaving the metal in the bath at least until a sediment has accumulated on the surface of the metal, and removing it from the bath for desired subsequent 40 treatment. 45
5. The process of treating high speed steel, which consists of immersing it in a molten bath of substantially seven parts lead and one part copper for a period of time proportional to about twenty minutes for a piece one-half inch in thickness, at a temperature between the fusing point of the bath and 1800 degrees Fahrenheit. 50

In witness whereof, I hereunto subscribe my name this 28th day of April A. D., 1923. 55

HERMAN J. BIEFANG.